

## [54] SYNTHETIC THERMOPLASTIC MULTIFILAMENT YARNS

[75] Inventors: **Etuzou Omura; Toshio Minami; Tetsuhiro Kusunose**, all of Nobeoka, Japan[73] Assignee: **Asahi Kasei Kogyo Kabushiki Kaisha**, Osaka, Japan[22] Filed: **June 19, 1972**[21] Appl. No.: **264,104**

## [30] Foreign Application Priority Data

|                |       |          |
|----------------|-------|----------|
| June 22, 1971  | Japan | 46-44504 |
| Sept. 20, 1971 | Japan | 46-72508 |
| Dec. 5, 1971   | Japan | 46-87585 |
| Dec. 5, 1971   | Japan | 46-87586 |
| Dec. 5, 1971   | Japan | 46-87587 |

[52] U.S. Cl. **57/153**, 117/7, 117/66, 117/138.8 E, 117/138.8 N, 117/138.8 F, 117/139.5 A, 117/139.5 CQ, 252/8.9, 260/31.2 R, 260/33.6 UA[51] Int. Cl. **D02g 3/36**, B32b 27/02[58] Field of Search... **117/138.8 N, 138.8 F, 138.8 E, 117/139.5 A, 139.5 CQ, 66, 7; 260/31.2 R, 23, 33.6 UA; 252/8.6, 8.9; 57/140 C, 153**

[56]

## References Cited

## UNITED STATES PATENTS

|           |         |                     |             |
|-----------|---------|---------------------|-------------|
| 2,253,146 | 8/1941  | Spragel .....       | 117/138.8   |
| 2,727,835 | 12/1955 | Barrett .....       | 117/138.8   |
| 2,819,189 | 1/1958  | Suen et al. ....    | 117/138.8 X |
| 2,974,066 | 3/1961  | Macura et al. ....  | 117/138.8 X |
| 3,003,987 | 10/1961 | Hager et al. ....   | 117/139.5 X |
| 3,476,581 | 11/1969 | Weitzel et al. .... | 117/139.5 X |
| 3,518,184 | 6/1970  | Potter .....        | 117/138.8 X |
| 3,560,382 | 2/1971  | Finch .....         | 117/138.8   |
| 3,639,235 | 2/1972  | Karg .....          | 252/8.9     |

Primary Examiner—William D. Martin

Assistant Examiner—Sadie L. Childs

Attorney, Agent, or Firm—Burgess, Dinklage &amp; Sprung

[57]

## ABSTRACT

Synthetic thermoplastic multifilament yarns with improved quality in coherency and smoothness having at most 100 twists per meter carrying about 0.5 to 3.0 percent, based on the weight of the yarns, of a treating agent comprising essentially a lubricating agent, a self-emulsifying phosphorous-containing surface active agent and a polyacrylic sizing agent, the polyacrylic size being present in about 0.02 to 0.25 percent, based on the weight of the yarns.

9 Claims, 4 Drawing Figures

## POLYACRYLIC SIZING AGENT



PATENTED DEC 24 1974

3,855,776

SHEET 1 OF 2

POLYACRYLIC SIZING AGENT

*Fig. 1*



*Fig. 2*



PATENTED DEC 24 1974

3,855,776

SHEET 2 OF 2



Fig. 3



Fig. 4

# SYNTHETIC THERMOPLASTIC MULTIFILAMENT YARNS

## BACKGROUND OF THE INVENTION

### 1. Field of the Invention

This invention relates to a novel synthetic thermoplastic multifilament yarn having good coherency and smoothness, a treating agent and a process for producing such a yarn.

### 2. Description of the Prior Art

At present, commonly practised methods for obtaining synthetic thermoplastic multifilaments having good coherency include steps such as imparting twist to drawn filaments or yarns or applying a viscous spinning oil or finishing oil to filaments or yarns. However, the coherency of such yarns is insufficient especially for warps. Therefore, in order to obtain good coherency of yarns an additional step such as giving at least 200 twists per meter to the yarns or sizing the yarns prior to weaving is required. In such a sizing step polyvinyl alcohols and maleic acid copolymers are usually employed alone or in combination as the sizing agent. Methods are already available for the omission of such twisting and sizing steps. For example, Japanese Patent 534,120 describes a treating agent comprising mainly a conventional spinning oil and a melamine resin or a urea resin. Japanese Patent 576,925 refers to ethylene-vinyl acetate copolymers as the treating agent. Japanese Patent 580,330 uses an emulsion of reaction products of a polyethylene with a polyolefin oxide and Japanese Patent Publication No. 15576/1969 also uses an emulsion of ethylene-acrylic acid copolymers. These methods all relate to the application of an emulsion of a resin and a sizing agent to filaments or yarns in the spinning process for obtaining the coherency. Furthermore, Japanese Patent Publication No. 3319/1971 and Japanese Patent 583,530 describe rendering filaments or yarns coherent only with a spinning oil comprising mainly a wax or a glyceride. All these treating methods may omit the sizing treatment in the spinning process but require twisting of yarns about 200 to 300 twists per meter before weaving, which disadvantageously results added in cost.

The present inventors have made extensive research on production of synthetic thermoplastic multifilament yarns or non-sized and non-twisted yarns useful as warps without any sizing and twisting treatment and initially polyacrylic sizing agents were applied to undrawn polyamide filaments or yarns and then the filaments or yarns were drawn. However, it is found the filaments or yarns thus obtained are not suitable for practical purposes because of the following disadvantages;

- a. The treating agent comprising a polyacrylic sizing agent as the principal component may not be uniformly applied to undrawn filaments due to high viscosity of the emulsion.
- b. The viscous materials stick to yarn-carrying devices such as guides, godet rolls and hinder the travelling of filaments or yarns.
- c. Due to hydrophilicity of the treating agent compared with a conventional spinning oil the package of undrawn filaments or yarns is deformed and it is difficult to wind up filaments or yarns to a package of predetermined size.
- d. The undrawn filaments or yarns tend to stick to one another and to a yarn-winding drum, and result in poor unreeling quality.

e. The treating agents sticking on undrawn filaments or yarns tend to come off in the drawing process due to abrasion on yarn-carrying devices such as guides, feed rolls, drawing pins and drawing rolls, and hinder the travelling of filaments or yarns thereby resulting in breakage of the individual filaments and fluff after producing.

f. In the drawing process coefficients of dynamic friction of the filaments or yarns become higher than those with a conventional spinning oil and hinder the travelling of filaments or yarns thereby resulting in breakage of the individual filaments and fluff after producing.

Thus, the method of applying a sizing agent to undrawn filaments or yarns in the spinning process, i.e., before drawing, is hardly practical because of the above-described disadvantages.

Accordingly, it is a primary object of this invention to provide novel weaving warps having good coherency and smoothness in the spinning process.

It is another object of this invention to omit the twisting and sizing processes conventionally required for imparting coherency and smoothness to filaments or yarns prior to weaving and to remarkably increase the speed of warping.

It is a further object of this invention to reduce the amount of sizing agents adhering to filaments and to abbreviate or omit the scouring process.

It is a still further object of this invention to provide weaving warps having good flexibility and softness which completely avoid the prior art pears and cracks due to stiffness of the conventionally sized yarns and which give improved quality textiles or fabrics.

Other objects and advantages will become apparent from the ensuing description.

## THE INVENTION

The present invention provides synthetic thermoplastic multifilament yarns of improved coherency and smoothness having at most 100 twists per meter carrying about 0.5 to 3.0 percent, based on the weight of the yarns, of a treating agent comprising essentially a lubricating agent, a self-emulsifying phosphorus-containing surface active agent and a polyacrylic sizing agent, the polyacrylic size being present in about 0.02 to 0.25 percent, based on the weight of the yarns.

In the drawings;

FIG. 1 is a triangular diagram, illustrative of a preferable composition of the lubricating agent, the self-emulsifying phosphorus-containing surface active agent and the polyacrylic sizing agent.

FIG. 2 is a diagram, illustrative of the relationship between the amount of polyacrylic sizing agents adhering to filaments and the fluff length on cutting a yarn.

FIG. 3 is a schematic view, illustrative of the method of measuring the fluff length, and

FIG. 4 is a schematic view, illustrative of the fluff length where the filaments of a yarn are loosened.

Examples of suitable lubricating agents to be used in this invention include mineral oils, lower alcohol esters having 1 to 8 carbon atoms of higher aliphatic carboxylic acids having 12 to 20 carbon atoms, higher alcohol esters having 12 to 20 carbon atoms of higher aliphatic carboxylic acids having 12 to 20 carbon atoms and mixtures thereof.

These lubricating agents may be classified broadly into two groups according to the kind of filaments or

yarns to which the lubricating agents are applied. For the warping process which is operated at a rate of more than 100 meters per minute, one group includes white spindle oils, liquid paraffins, the lower alcohol esters of the higher carboxylic acids such as methyl ricinolate, 5 methyl oleate, methyl stearate, isopropyl myristate, iso-propyl palmitate, n-butyl oleate, n-butyl laurate, n-butyl stearate, epoxybutyl stearate, isoamyl stearate, n-octyl palmitate, n-octyl laurate, n-octyl oleate, n-octyl stearate and mixtures thereof. The Redwood viscosity at 30°C. of these lubricants is preferably in the range of from about 40 to about 100 seconds. For the warping process which is operated at a rate of 100 meters per minute or thereabout, the other group includes white spindle oils, liquid paraffins, the higher alcohol 15 esters of the higher carboxylic acids such as lauryl laurate, tetradecyl laurate, cetyl laurate, oleyl laurate, stearyl laurate, lauryl myristylate, tetradecyl myristylate, cetyl myristylate, oleyl myristylate, stearyl myristylate, lauryl palmitate, tetradecyl palmitate, cetyl palmitate, oleyl palmitate, etearyl palmitate, lauryl stearate, tetradecyl stearate, cetyl stearate, oleyl stearate, stearyl stearate, and mixtures thereof. The Redwood viscosity at 30°C. of these lubricants is preferably in the range of from about 100 to about 500 seconds. 20 25

The amount of these lubricating agents varies depending on the kind of self-emulsifying phosphorus-containing surface active agents and polyacrylic sizing agents and of the filament or yarns to be treated and is preferably in the range of from about 5 to 68 percent on the weight of the treating agent. (17) (18)

Exemplary self-emulsifying phosphorus-containing surface active agents include the compounds having the following formulae;





and any mixture of these compounds wherein  $n$  represents 1 to 100;  $\text{R}^1$  represents an alkyl group or alkyl-phenyl group having 8 to 30 carbon atoms; and  $\text{R}^2$  represents an alkyl group having 1 to 22 carbon atoms, an allyl group or an allylalkyl group having 4 to 25 carbon atoms.

The surface active agents act as emulsifiers, cohesive agents and antistatic agents.

These self-emulsifying phosphorus-containing surface active agents are employed in an amount of about 30 to 80 percent based on the weight of the treating. Amounts of less than 30 percent by weight of the surface active agents render the emulsion of the treating agent less stable. On the other hand when the amount is more than 80 percent by weight, the viscosity of the emulsion of the treating agent remarkably increases and an even and uniform application of the treating agent to filaments or yarns becomes difficult.

It is also preferred that the hydrophilic-lipophilic balance (hereinafter referred to as HLB) of the self-emulsifying phosphorus-containing surface active agent is from about 4 to 15.

The HLB of more than 15 or less than 4 results in unsatisfactory emulsification of the treating agent.

The HLB is represented by a number of 0 to 20. The numbers closer to 20 indicate a higher lipophilicity of the surface active agent and those closer to 0 indicate a higher hydrophilicity.

Examples of suitable polyacrylic sizing agents which may be employed in this invention include polyacrylic acid, sodium polyacrylate, lower alkyl esters of partially saponified polyacrylic acids, lower alkyl esters of partially saponified polyacrylic acid copolymers, salts of polymethacrylic acid, polyacrylamide, acrylonitrile copolymers and saponified copolymers of vinyl acetate and a variety of acrylic monomers. The degree of polymerization of the acrylic polymers is preferably from about 100 to 2,000. The polyacrylic sizing agents should be determined according to the kind of filaments to be treated.

These polyacrylic sizing agents are used in an amount of from about 2 to about 15 percent, and preferably from about 4 to 8 percent based on the weight of the treating agent. When the amount is less than 2 percent by weight inadequate coherency will be given to filaments or yarns. On the other hand, amounts of more than about 15 percent by weight of polyacrylic sizing agents render the viscosity of the emulsion of the treating agent too high to obtain an even and uniform application of the treating agent to filaments or yarns and furthermore the sizing agents adhering to the filaments or yarns come off and reduce workability.

The treating agents according to this invention may additionally contain antistatic agents in conventionally employed amounts.

It is preferred that the amount of the treating agent adhering to filaments or yarns is from about 0.5 percent to 3.0 percent based on the weight of the filaments or yarns. When the amount is less than 0.5 percent by

weight, yarns having a desired good coherency may not be obtained. On the other hand, amounts of more than 3.0 percent by weight of the treating agent unusually increase the coefficient of friction of filaments or yarns and consequently the spinning and drawing processes cannot be smoothly operated. Furthermore, as the treating agent adhering to filaments or yarns comes off by the motion of a weaving machine in the weaving process, the efficiency of weaving is reduced and the quality of fabrics obtained from the yarns is degraded.

Since any practical method of measuring the coherency of multifilament yarns has not been established yet, the coherency is represented by the fluff length on cutting a yarn.

On a device as illustrated in FIG. 3, a 0.5m. sample yarn 1 is set and to the end of the yarn a weight 3 of 50g. is applied. After five minute loading, the yarn is cut with scissors 2 at a point 5 cm. from the weight. Subsequently, as shown in FIG. 4, the fluff length 1 where the filaments of the longer yarn 1 are loosened is measured.

A longer fluff length indicates a power coherency and a shorter fluff length indicates a better coherency. In this connection, the fluff length of a conventionally sized yarn is 15mm. and that of a conventionally non-sized yarn is 130mm.

According to a general idea the coherency may be improved with increased amounts of sizing agents. On the contrary, it has now been found that there exists an optimum range in the relationship between the amount of sizing agents adhering to filaments or yarns and the coherency.

In this invention the amount of polyacrylic sizing agents adhering to filaments or yarns is preferably from about 0.02 to 0.25 percent and more preferably from about 0.075 to 0.175 percent based on the weight of the filaments or yarns. As is clear from FIG. 2, amounts of more than about 0.25 percent by weight or less than about 0.02 percent by weight of sizing agents adhering to filaments or yarns give a fluff length of 50mm. or more and thus reduce not only the coherency but also the efficiency of weaving. A more preferred fluff length of about 30mm. is obtained with amounts of about 0.075 to 0.175 percent by weight of filaments or yarns. When the amount is more than about 0.25 percent by weight the coherency is decreased and furthermore the sizing agents come off on yarn-carrying devices in the winding, drawing and twisting processes and workability is remarkably diminished. Even if undrawn filaments are wound up, the drawing of the filaments become impossible due to an unusual increase in the coefficient of dynamic friction of the filaments.

In order to adjust the amount of polyacrylic sizing agents adhering to filaments to the range of from about 0.02 to 0.25 percent based on the weight of the filaments or yarn it is preferred to use the treating agent in a concentration of about 10 to 25 percent by weight and a winding rate of filaments or yarns of from about 600 to 5,000 m./min.

FIG. 1 is a triangular diagram, illustrative of the compositions of a mineral oil having a Redwood viscosity at 30°c. of 150 seconds as the lubricating agent, a polyethylene glycol ester of alkylphosphate having a HLB of 6.9 (Trade mark: "GAFAC GB-520" made by Toho Chemical Ind. Co., Ltd.) and a polyacrylic sizing agent (Trade mark: "PLUSSIZE J<sub>4</sub>" made by Gao Chemical

Ind. co., Ltd.), which give good coherency to filaments or yarns according to this invention.

Exemplary synthetic thermoplastic materials constituting the filaments or yarns to be subjected to the treatment of this invention include polyamides, polyesters and polypropylenes.

The multifilament yarns having been treated with the treating agents according to this invention have excellent antistatic properties and good efficiency of weaving as well as good coherency and smoothness. The textiles or fabrics obtained from the yarns are soft to the touch and free from disadvantages such as pear drops and cracks. Moreover, the yarns have excellent water resistance and are suitable not only for ordinary shuttle weaving machines but also for water-jet looms which have rapidly become popular. Scouring can also be easily effected with the yarns by choosing a sizing agent suitable for the yarns. Scouring with the yarns according to this invention is superior to that with the conventionally sized yarns which have been treated with a treating agent mainly containing a sizing agent.

The treatment with the treating agent according to this invention is effected by the conventional methods, for example, by immersing filaments or yarns in a bath of an emulsion of the treating agent or applying the treating agent to filaments or yarns with an oiling roll or a spray.

The treating agent may be uniformly applied to filaments or yarns in the filament producing processes, especially in the spinning process, but also in any process after spinning, for example, in a process with a drawing machine, a cone winder or a cheese winder prior to weaving, by the conventional methods at room temperature.

The treating agent of this invention may be employed for weaving warps as previously stated but may also be employed for weaving woofs, tricot yarns and all other

yarns which require coherency. For example it is possible to apply the treating agent to modified section yarns, nep yarns, thick-and-thin yarns by an uneven drawing, conjugated yarns and other novel yarns which are generally considered inferior in coherency.

This invention will be further illustrated by the following non-limiting examples.

#### EXAMPLE 1

10 To a melt-spun, undrawn, semi-dull nylon 6 multifilament yarn consisting of 24 filaments having a denier of 210 there were independently applied to emulsions of 15 treating agents A, B and C set forth below by rolls of spinning oil supplying devices according to an ordinary method when taken up at a rate of 1,000 meters per minute so that the amount of the treating agent adhering to the undrawn yarn was about 1.5 percent based on the weight of the yarn. After completion of the treatment the undrawn yarn was drawn 3 times by usual 20 drawing and twisting machines and wound up on bobbins to give a multifilament yarn having 15 twists per meter and consisting of 24 filaments having a denier of 70. Then the multifilament yarns treated with the treating agents A, B and C were subjected to rough warping 25 without another twisting and sizing, and subsequently to beaming, warp passing and water-jet looming processes. (Thus, 50 pieces of taffets textile fabrics were obtained each having a width of 120 cm. and a length of 50 m.)

30 Separately, the multifilament yarn (C) was sized with a polyacrylate sizing agent by a slasher sizing machine without another twisting to give the multifilament yarn (D). Then the yarn (D) was subjected to beaming, warp passing and water-jet looming processes and 35 50 pieces of taffeta textile fabrics were obtained. The features of these yarns (A), (B), (C) and (D) measured in the drawing, weaving and finishing processes are set forth in Table 1.

##### Composition of treating agent A according to this invention

|                                                                                                                     |             |
|---------------------------------------------------------------------------------------------------------------------|-------------|
| a. Liquid paraffin having a Redwood viscosity at 30°C of 60 seconds                                                 | 44 weight % |
| b. Alkylphosphate of polyethylene glycol ether<br>(Trade mark: "GAFAC GB-520" made by Toho Chemical Ind. Co., Ltd.) | 50          |
| c. Polyacrylate sizing agent<br>(Trade mark: "PUSSIZE 208C" made by Gao Chemical Ind. Co., Ltd.)                    | 6           |

##### Composition of treating agent B according to this invention

|                                                                                                                     |             |
|---------------------------------------------------------------------------------------------------------------------|-------------|
| a. Liquid paraffin having a Redwood viscosity at 30°C of 250 seconds                                                | 44 weight % |
| b. Alkylphosphate of polyethylene glycol ether<br>(Trade mark: "GAFAC GB-520" made by Toho Chemical Ind. Co., Ltd.) | 50          |
| c. Polyacrylate sizing agent<br>(Trade mark: "PLUSSIZE 208C" made by Gao Chemical Inc. Co., Ltd.)                   | 6           |

##### Composition of treating agent C according to a conventional method

|                                                                                       |             |
|---------------------------------------------------------------------------------------|-------------|
| a. Liquid paraffin having a Redwood viscosity at 30°C of 100 seconds                  | 60 weight % |
| b. Sperm alcohol (EO)<br>(Trade mark: AC-301" made by Sanyo Chemical Inc. Co., Ltd.)  | 30 weight % |
| c. Sulfated oil of sperm alcohol<br>(Trade mark: "AK-37" made by Kao Atlas Co., Ltd.) | 10          |

The treating agents A, B and C, each independently were dispersed in water to obtain emulsions A, B and C with a concentration of the treating agent of 16 weight %.

rate of cylinder of 30 r.p.m. (Temperature: 20°C., RH: 65 percent)

8. Gumming: The falling off of treating agent, adhering to filaments or yarns due to looming motion is

Table 1

| Features                                                        | Treatment according to this method |       | Treatment according to conventional method |           |
|-----------------------------------------------------------------|------------------------------------|-------|--------------------------------------------|-----------|
|                                                                 | (A)                                | (B)   | non-sized (C)                              | Sized (D) |
| Amount of treating agent adhering to yarns (weight %)           | 1.4                                | 1.3   | 1.2                                        | 1.3       |
| Amount of polyacrylic sizing agent adhering to yarns (weight %) | 0.08                               | 0.078 | 0                                          | 5.5       |
| <u>Process</u>                                                  |                                    |       |                                            |           |
| <u>Drawing process</u>                                          |                                    |       |                                            |           |
| (1) Drawing yield (%)                                           | 98                                 | 96    | 95                                         | 95        |
| (2) Fallen off materials                                        | 5                                  | 4-5   | 5                                          | 5         |
| (3) Generated static electricity (V.)                           | 2,500                              | 2,600 | 2,700                                      | 2,700     |
| (4) Pirn unreeling ability (g.)                                 | 6.0                                | 9.0   | 8.0                                        | 8.0       |
| (5) Coherency (mm.)                                             | 29                                 | 27    | 134                                        | 134       |
| <u>Weaving process</u>                                          |                                    |       |                                            |           |
| (6) Coherency (mm.)                                             | 29                                 | 27    | 134                                        | 26        |
| (7) Smoothness ( $\mu$ s)                                       | 0.275                              | 0.278 | 0.231                                      | 0.252     |
| do. ( $\mu$ d)                                                  | 0.140                              | 0.200 | 0.138                                      | 0.195     |
| (8) Gumming                                                     | 4-5                                | 4-5   | 5                                          | 4-5       |
| (9) Rate of weaving operation (%)                               | 92                                 | 93    | 40                                         | 92        |
| <u>Finishing process</u>                                        |                                    |       |                                            |           |
| (10) Scouring ability                                           | 4-5                                | 5     | 5                                          | 3-4       |
| (11) Defects of weaving warps                                   | 4-5                                | 4-5   | 2-3                                        | 3-4       |
| (12) Yield of first grade textile fabrics (%)                   | 94                                 | 95    | 61                                         | 90        |

## Note:

1. Drawing yield (%): Yield of first grade multifilament yarns based on all drawn multifilament yarns  
 2. Fallen off material: Degree of amounts of adhesives on film-forming materials which fall off from multifilament yarns on the yarn-conveying devices of drawing machine is evaluated as follows:

40

- 1: Too much accumulated for operating drawing  
 2: Large amount accumulated  
 3: Much accumulated  
 4: A little accumulated but drawing not hindered  
 5: No fallen off material

3. Generated static electricity (V.): When undrawn multifilament yarns are subjected to drawing by a drawing machine at a rate of 600 meters per minute, generated static electricity at each of devices of a drawing machine such as feed rolls, drawing pins and pirns is measured by a static electricity measuring instrument made by Kasuga Electric Co., Ltd. The maximum value during the drawing is given.

45

4. Pirn unreeling ability (g.): Tension of unreeling from a pirn is measured.  
 (5)&(6) Coherency (mm.): On a device illustrated in FIG. 3, a 0.5 m. sample yarn is set and to end of the yarn a weight of 50 g. is applied. After 5 minutes loading, the yarn is cut with scissors at the point 5 cm. from the weight. Subsequently, as shown in FIG. 4, the length where filaments are loosened is measured.

50

7. Smoothness: Smoothness is measured by a friction coefficient measuring device according to the Roe-der method with a weight of 500 mg. at a rotating

called "Gumming." amounts of adhesives or film-forming materials which fall off from multifilament yarns is evaluated as follows;

- 1: Accumulated too much for operating weaving  
 2: large amount accumulated  
 3: Much accumulated  
 4: A little accumulated but weaving not hindered  
 5: No gumming

9. Rate of weaving operation (percent): Rate of weaving operation from the beginning to the completion of weaving excluding the factors which are not directly related to weaving, e.g., waiting time, etc.

10. Scouring ability: amounts of lubricating agents and polyacrylic sizing agents which are removed off during the scouring process before dyeing is evaluated as follows;

- 1: No removal at all  
 2: Removed but much remained  
 3: About 50 weight percent removed and about 50 weight % remained  
 4: A little remained and most removed  
 5: Completely removed

11. Defects of weaving warps: Degree of causing defects of weaving warps such as pear drops and cracks is evaluated as follows;

- 1: Too much appeared for use as textile fabrics  
 2: Considerable defects  
 3: A little appeared  
 4: A little appeared but usable as textile fabrics  
 5: No defect at all

12. Yield of first grade textile fabrics (percent): To

55

60

65

all woven textile fabrics the ratio of pieces which are accepted as first grade textile fabrics.

#### EXAMPLE 2

To a melt-spun, undrawn, polyethylene terephthalate multifilament yarn consisting of 24 filaments having a denier of 225 there were independently applied the emulsions of treating agents A, B and C set forth below in the same manner as in Example 1 when taken up at a rate of 1,000 meters per minute so that the amount of the treating agent was about 1.5 percent based on the weight of the yarn. After completion of the treatment the undrawn yarn was hot drawn 3 X by usual drawing and twisting machines and wound up on bobbins to give a yarn having 15 twists per meter and con-

5 10 15

sisting of 24 filaments having a denier of 75. Then the multifilament yarns treated with the treating agents A, B and C were subjected to rough warping without another twisting and sizing, and subsequently to beaming, warp passing and water-jet looming. Thus 50 pieces of taffeta textile fabrics were obtained.

Separately, the multifilament yarn (C) was sized with a polyacrylate sizing agent by a slusher sizing machine without another twisting to give the multifilament yarn (D). Then the yarn (D) was subjected to beaming, warp passing and water-jet looming and 50 pieces of taffeta textile fabrics were obtained. The features of these yarns (A), (B), (C) and (D) measured in the drawing, weaving and finishing process are set forth in Table 2.

Table 2

| Features                                                        | Treatment according to this method |       | Treatment according to conventional method |           |
|-----------------------------------------------------------------|------------------------------------|-------|--------------------------------------------|-----------|
|                                                                 | (A)                                | (B)   | non-sized (C)                              | Sized (D) |
| Amount of treating agent adhering to yarns (weight %)           | 1.5                                | 1.5   | 1.1                                        | 1.0       |
| Amount of polyacrylic sizing agent adhering to yarns (weight %) | 0.15                               | 0.15  | 0                                          | 6.5       |
| <u>Process</u>                                                  |                                    |       |                                            |           |
| <u>Drawing process</u>                                          |                                    |       |                                            |           |
| (1) Drawing yield (%)                                           | 95                                 | 93    | 94                                         | 94        |
| (2) Fallen off materials                                        | 4-5                                | 4-5   | 5                                          | 5         |
| (3) Generated static electricity (V.)                           | 2,000                              | 3,100 | 3,600                                      | 3,600     |
| (4) Pern unreeeling ability (g.)                                | 7.1                                | 9.6   | 8.3                                        | 8.3       |
| (5) Coherency (mm.)                                             | 34                                 | 27    | 141                                        | 141       |
| <u>Weaving process</u>                                          |                                    |       |                                            |           |
| (6) Coherency (mm.)                                             | 34                                 | 27    | 141                                        | 28        |
| (7) Smoothness ( $\mu$ s)                                       | 0.281                              | 0.281 | 0.291                                      | 0.263     |
| do. ( $\mu$ d)                                                  | 0.151                              | 0.214 | 0.148                                      | 0.203     |
| (8) Gumming                                                     | 4-5                                | 4-5   | 5                                          | 4-5       |
| (9) Rate of weaving operation(%)                                | 91                                 | 90    | 51                                         | 89        |
| <u>Finishing process</u>                                        |                                    |       |                                            |           |
| (10) Scouring ability                                           | 4-5                                | 4-5   | 5                                          | 3-4       |
| (11) Defects of weaving warps                                   | 4-5                                | 4-5   | 2-3                                        | 3-4       |
| (12) Yield of first grade textile fabrics (%)                   | 94                                 | 91    | 71                                         | 93        |

## EXAMPLE 3

To a melt-spun, undrawn, semi-dull nylon 6 multifilament yarn consisting of 17 filaments having a denier of 210 there was applied the emulsion of treating agent shown below by rolls when taken up at a rate of 1,000 meters per minute so that the amount of the treating agent adhering to the undrawn yarn was about 1.5 percent based on the weight of the yarn. After completion of the treatment, the wound, undrawn yarn was drawn 3 X by ordinary drawing and twisting machines, and wound up on bobbins to give a multifilament yarn having 15 twists per meter and a fluff-length on cutting a yarn of 28 mm. and consisting of 17 filaments having a denier of 70. During the above-described spinning, winding-up, drawing and twisting processes, there was observed no falling off of the polyacrylic sizing agent adhering to the yarn and the yarn traveled very smoothly on the yarn-carrying devices. Yield of first grade multifilament yarns was 90 percent. Then the multifilament yarn was subjected to rough warping process without another twisting of more than 100 twists per meter, and sizing, and subsequently to beaming, warp passing and water-jet looming. Thus, 50 pieces of taffeta textile fabrics were obtained. During the weaving process there was observed no falling off of the sizing agent. Rate of weaving operation was 96 percent, and this rate was equal to or higher than that with a conventionally sized yarn. The textile fabrics thus obtained were almost free from pear drops and cracks. Also scouring ability was good and yield of first grade textile fabrics was 91 percent, which was equal to or higher than that with a conventionally sized yarn.

## EXAMPLE 4

To the same melt-spun, undrawn, semi-dull nylon 6 multifilament yarn as in Example 3 there was independently applied the same emulsion of treating agent as in Example 3 and the same emulsion of treating agent C as in Example 1 by rolls when taken up at a rate of 1,000 meters per minute and subsequently the undrawn 10 yarn was drawn 3X by ordinary drawing machines to give a multifilament yarn consisting of 17 filaments having a denier of 70. Falling off of the treating agent occurred to a small extent during the drawing process and drawing yield was good. Then the drawn yarn was 15 given a variety of twists as set forth in Table 3. The twisted yarns were subjected to warping process which was effected at a rate of 150 meters per minute, and further to beaming, reeling, heald passing and water-jet looming. Thus, 20 pieces of taffeta textile fabrics were 20 obtained using, as woofs, non-twisted, non-sized nylon 6 yarns consisting of 24 filaments having a denier 70. The results are shown in Table 3.

25 As is clear from Table 3, the yarns treated with the treating agent C of Example 1 according to a conventional method require at least 100 twists per meter for weaving while those treated with the treating agent of Example 3 having less than about 100 twists per meter permit weaving. In other words, the yarns according to this invention do not require twisting and are economically more advantageous than the non-twisted sized 30 yarns or the twisted non-sized yarns having at least 100

## Composition of treating agent

|                                                                                                                                         |             |
|-----------------------------------------------------------------------------------------------------------------------------------------|-------------|
| a. Liquid paraffin having a Redwood viscosity at 30°C. of 250 seconds                                                                   | 40 weight % |
| b. Alkylphosphate of polyethylene glycol ether having a HLB of 6.9<br>(Trade mark: "GAFAC GB-520" made by Toho Chemical Inc. Co., Ltd.) | 50          |
| c. Alkylimidazoline<br>(Trade mark: "ELECTROSTRIPPER C"<br>made by Kao Atlas Co., Ltd.)                                                 | 4           |
| d. Polyacrylate sizing agent<br>(Trade mark: "PLUSSIZE 208C"<br>made by Gao Chemical Ind. Co., Ltd.)                                    | 6           |

The treating agents was dispersed in water to obtain an emulsion having a concentration of treating agent of 16%.

50 twists per meter according to the conventional method. Similar results are obtained with polyester multifilament yarns and polypropylene yarns.

Table 3

| Number<br>of<br>twists<br>per meter | Results according to this invention                     |                                                  |                                        |                                   | Results according to the conventional method            |                                                  |                                        |                                   |
|-------------------------------------|---------------------------------------------------------|--------------------------------------------------|----------------------------------------|-----------------------------------|---------------------------------------------------------|--------------------------------------------------|----------------------------------------|-----------------------------------|
|                                     | Treating<br>agent<br>adhering<br>to yarns<br>(weight %) | Fluff<br>length on<br>cutting<br>a yarn<br>(mm.) | Rate of<br>weaving<br>operation<br>(%) | Quality<br>of<br>woven<br>fabrics | Treating<br>agent<br>adhering<br>to yarns<br>(weight %) | Fluff<br>length on<br>cutting<br>a yarn<br>(mm.) | Rate of<br>weaving<br>operation<br>(%) | Quality<br>of<br>woven<br>fabrics |
| 0                                   | 1.2                                                     | 36                                               | 92                                     | Excellent                         | 1.0                                                     | 130                                              | Impossible                             | —                                 |
| 15                                  | 1.3                                                     | 33                                               | 96                                     | do.                               | 1.0                                                     | 125                                              | do.                                    | —                                 |
| 30                                  | 1.2                                                     | 31                                               | 93                                     | Good                              | 0.9                                                     | 110                                              | do.                                    | —                                 |
| 50                                  | 1.4                                                     | 28                                               | 94                                     | Excellent                         | 1.0                                                     | 94                                               | do.                                    | —                                 |
| 70                                  | 1.3                                                     | 27                                               | 91                                     | do.                               | 1.2                                                     | 96                                               | do.                                    | —                                 |
| 100                                 | 1.4                                                     | 29                                               | 95                                     | Good                              | 1.1                                                     | 88                                               | 65                                     | Poor                              |
| 120                                 | 1.2                                                     | 31                                               | 94                                     | Excellent                         | 0.9                                                     | 83                                               | 87                                     | Good                              |
| 150                                 | 1.3                                                     | 26                                               | 95                                     | do.                               | 0.9                                                     | 75                                               | 91                                     | Excellent                         |
| 200                                 | 1.3                                                     | 24                                               | 97                                     | do.                               | 1.1                                                     | 71                                               | 94                                     | do.                               |

## EXAMPLE 5

To the same melt-spun, undrawn, semi-dull nylon 6 multifilament yarn as in Example 3 there was applied the same emulsion of treating agent as in Example 3 when taken up at a rate of 1,000 meters per minute by rolls having a variety of rotating rates so that the amount of treating agent adhering to the yarn was varied, and then the undrawn yarn was drawn 3 $\times$  by ordinary drawing machines to give a multifilament yarn 10 consisting of 17 filaments having a denier of 70. The yarn was subjected to warping at a rate of 150 meters per minute, and further to beaming reeling, heald passing and water-jet looming. Using, as woofs, non-

become remarkable and workability is reduced. Furthermore, the coherency is gradually decreased and the rate of weaving operation is diminished. Similar results are obtained with polyester multifilament yarns and polypropylene multifilament yarns.

Also as is understood from Table 4, the rate of weaving operation is kept above 90 percent only when the fluff length on cutting a yarn is below 50 mm. as long as breakage of filaments or yarns during the drawing process is not brought about too often. Practically it is desirable that the rate of weaving is at least 90%. Accordingly, in order to obtain such high rates of weaving operation the maximum fluff length on cutting a yarn is about 50 mm.

Table 4

| Polyacrylic<br>sizing agent<br>adhering<br>to yarns<br>(weight %) | Workability                                                       | Number of<br>breaks per<br>Kg. of filaments<br>during drawing | Fluff length<br>on cutting<br>a yarn<br>(mm.) | Weaving                                |                                   |
|-------------------------------------------------------------------|-------------------------------------------------------------------|---------------------------------------------------------------|-----------------------------------------------|----------------------------------------|-----------------------------------|
|                                                                   |                                                                   |                                                               |                                               | Rate of<br>weaving<br>operation<br>(%) | Quality<br>of<br>woven<br>fabrics |
| 0                                                                 | Winding up was impossible                                         | —                                                             | —                                             | —                                      | —                                 |
| 0.01                                                              | No problem                                                        | 0.02                                                          | 68                                            | 50                                     | Poor                              |
| 0.02                                                              | do.                                                               | 0.01                                                          | 50                                            | 90                                     | Good                              |
| 0.03                                                              | do.                                                               | 0.03                                                          | 45                                            | 92                                     | Excellent                         |
| 0.05                                                              | do.                                                               | 0.02                                                          | 38                                            | 96                                     | do.                               |
| 0.10                                                              | do.                                                               | 0.01                                                          | 27                                            | 95                                     | do.                               |
| 0.15                                                              | do.                                                               | 0.03                                                          | 27                                            | 96                                     | do.                               |
| 0.20                                                              | do.                                                               | 0.04                                                          | 35                                            | 94                                     | do.                               |
| 0.25                                                              | Polyacrylate sizing agent slightly<br>spattered during drawing    | 0.08                                                          | 50                                            | 91                                     | Good                              |
| 0.30                                                              | Polyacrylate sizing agent slightly<br>spattered during drawing    | 0.56                                                          | 79                                            | 45                                     | Poor                              |
| 0.50                                                              | Polyacrylate sizing agent excessively<br>spattered during drawing | 1.11                                                          | 136                                           | —                                      | Impossible                        |

twisted, non-sized nylon 6 yarns consisting of 24 filaments having a denier of 70, there were obtained 20 pieces of taffeta textile fabrics. The results are shown in Table 4.

As is clear from Table 4, there is an optimum relationship between the amount of polyacrylic sizing agent adhering to a yarn, the coherency and the rate of weaving operation. The optimum range of polyacrylic sizing agent is from about 0.02 to 0.25 percent based on the weight of the yarn. When the amount is less than 0.02 weight percent, good cohesion of yarns cannot be obtained due to insufficient adhesion by the sizing agent and the rate of weaving operation is very low. On the other hand, with amounts of more than 0.25 weight percent of the sizing agent falling off of the sizing agent

40 The procedure of Example 5 was repeated except that the amount of treating agent adhering to the yarn was varied. The results are shown in Table 5.

As is understood from Table 5, when the amount of treating agent adhering to yarns is less than about 0.5 weight percent it is difficult to wind up the undrawn multifilament yarn and good coherency cannot be obtained. On the other hand, amounts of more than 0.5 weight percent of the treating agent remarkably bring about falling off of the treating agent and workability is also remarkably reduced. Furthermore, the coherency is diminished with increased amounts of the polyacrylic sizing agent.

Table 5

| Treating<br>agent<br>adhering<br>to yarns<br>(weight %) | Workability                                                                                       | Number of<br>breaks per<br>Kg. of filaments<br>during drawing | Fluff length<br>on cutting<br>a yarn<br>(mm.) | Weaving                                |                                   |
|---------------------------------------------------------|---------------------------------------------------------------------------------------------------|---------------------------------------------------------------|-----------------------------------------------|----------------------------------------|-----------------------------------|
|                                                         |                                                                                                   |                                                               |                                               | Rate of<br>weaving<br>operation<br>(%) | Quality<br>of<br>woven<br>fabrics |
| 0                                                       | Winding up was impossible                                                                         | —                                                             | —                                             | —                                      | —                                 |
| 0.1                                                     | Winding up was rather difficult                                                                   | 0.05                                                          | 90                                            | —                                      | —                                 |
| 0.3                                                     | No problem                                                                                        | 0.01                                                          | 70                                            | 65                                     | Impossible                        |
| 0.5                                                     | do.                                                                                               | 0.03                                                          | 45                                            | 92                                     | Poor                              |
| 0.7                                                     | do.                                                                                               | 0.04                                                          | 34                                            | 94                                     | Excellent                         |
| 1.0                                                     | do.                                                                                               | 0.00                                                          | 31                                            | 92                                     | do.                               |
| 1.5                                                     | do.                                                                                               | 0.01                                                          | 27                                            | 95                                     | do.                               |
| 2.0                                                     | do.                                                                                               | 0.01                                                          | 29                                            | 93                                     | do.                               |
| 2.5                                                     | do.                                                                                               | 0.03                                                          | 27                                            | 96                                     | do.                               |
| 3.0                                                     | Small amount of treating agent adhering to yarns<br>fell off                                      | 0.04                                                          | 35                                            | 94                                     | Good                              |
| 5.0                                                     | Excessive amount of treating agent adhering to yarns<br>fell off and wound-up yarns were deformed | 0.56                                                          | 79                                            | 45                                     | Poor                              |

## EXAMPLE 7

To a melt-spun, undrawn, semi-dull nylon 6 multifilament yarn consisting of 17 filaments having a denier of 210 there were applied a variety of emulsions having a

polyacrylic sizing agent in the treating agent is from about 4 to 8 weight percent in terms of drawing and weaving. The preferred range of the alkylphosphate of polyethylene glycol ether in the treating agent is from about 30 to 80 weight percent.

Table 6

| Polyacrylic sizing agent (weight %) | Treating agent             |                                                        | Workability                                                   | Number of breaks per Kg. of filaments during drawing | Treating agent adhering to yarns (weight %) | Fluff length on cutting a yarn (mm.) | Weaving                       |                          |
|-------------------------------------|----------------------------|--------------------------------------------------------|---------------------------------------------------------------|------------------------------------------------------|---------------------------------------------|--------------------------------------|-------------------------------|--------------------------|
|                                     | Liquid paraffin (weight %) | Alkylphosphate of polyethylene glycol ether (weight %) |                                                               |                                                      |                                             |                                      | Rate of weaving operation (%) | Quality of woven fabrics |
| 0                                   | 40                         | 60                                                     | No problem                                                    | 0.01                                                 | 1.4                                         | 61                                   | —                             | Impossible               |
| 2                                   | 40                         | 58                                                     | do.                                                           | 0.02                                                 | 1.3                                         | 53                                   | 87                            | Good                     |
| 4                                   | 40                         | 56                                                     | do.                                                           | 0.03                                                 | 1.5                                         | 34                                   | 93                            | Excellent                |
| 6                                   | 40                         | 54                                                     | do.                                                           | 0.06                                                 | 1.4                                         | 28                                   | 95                            | do.                      |
| 8                                   | 40                         | 52                                                     | do.                                                           | 0.09                                                 | 1.3                                         | 38                                   | 96                            | do.                      |
| 10                                  | 40                         | 50                                                     | do.                                                           | 0.07                                                 | 1.6                                         | 48                                   | 90                            | Good                     |
| 15                                  | 40                         | 45                                                     | Polyacrylic sizing agent slightly spattered during drawing    | 0.12                                                 | 1.6                                         | 52                                   | 85                            | do.                      |
| 20                                  | 40                         | 40                                                     | Polyacrylic sizing agent excessively spattered during drawing | 7.30                                                 | 1.9                                         | 75                                   | —                             | Impossible               |
| 6                                   | 74                         | 20                                                     | Emulsification was too poor for use                           | —                                                    | —                                           | —                                    | —                             | —                        |
| 6                                   | 64                         | 30                                                     | Emulsification was slightly poor but usable                   | 0.01                                                 | 1.3                                         | 34                                   | 90                            | Excellent                |
| 6                                   | 54                         | 40                                                     | No problem                                                    | 0.01                                                 | 1.2                                         | 30                                   | 96                            | do.                      |
| 6                                   | 44                         | 50                                                     | do.                                                           | 0.02                                                 | 1.4                                         | 33                                   | 95                            | do.                      |
| 6                                   | 34                         | 60                                                     | do.                                                           | 0.03                                                 | 1.6                                         | 29                                   | 92                            | Good                     |
| 6                                   | 24                         | 70                                                     | do.                                                           | 0.00                                                 | 1.7                                         | 27                                   | 91                            | Excellent                |
| 6                                   | 14                         | 80                                                     | viscosity of emulsion was slightly high but usable            | 0.06                                                 | 1.9                                         | 25                                   | 89                            | do.                      |
| 6                                   | 4                          | 90                                                     | Viscosity of emulsion was too high for use                    | —                                                    | —                                           | —                                    | —                             | —                        |

Polyacrylic sizing agent: Trade mark, "PLUSSIZE 208C" made by Gao Chemical Ind. Co., Ltd.

Liquid paraffin having a Redwood viscosity at 30°C. of 250 seconds

Alkylphosphate of polyethylene glycol ether: Trade mark, "GAFAC GB-520" made by Toho Chemical Ind. Co., Ltd.

concentration of the treating agent of 16 weight percent set forth in Table 6 by rolls when taken up at a rate of 1,000 meters per minute and the undrawn yarn was drawn 3× by ordinary drawing and twisting machines to give a multifilament yarn having 15 twists per meter and consisting of 17 filaments having a denier of 70. Then the drawn multifilament yarn was subjected to warping which was effected at a rate of 150 meters per minute, without sizing, and further to beaming, reeling, heald passing and water-jet looming. Using, as woofs, non-twisted, non-sized nylon 6 yarns having 24 filaments having a denier of 70, there were obtained 20 pieces of taffeta textile fabrics. The results are shown in Table 6.

As is clear from Table 6 the optimum range of the

40 The procedure of Example 7 was repeated except that a variety of emulsions having a concentration of 45 the treating agent of 16 weight percent set forth in Table 7 were employed. The results are shown in Table 7.

45 As is shown in Table 7 the coherency does not vary much even when the Redwood viscosity of the liquid paraffin is changed from 40 to 500 seconds and the kinds of self-emulsifying phosphorus-containing surface active agents and polyacrylic sizing agents are changed. Multifilament yarns having a fluff length of 50 less than about 50 mm. can be easily obtained from such treating agents as set forth in Table 7.

Table 7

| Treating agent                |                                                               | Self-emulsifying surface active agent 50 weight % | Polyacrylic sizing agent 6 weight % | Treating agent adhering to yarns (weight %) | Fluff length on cutting yarn (mm.) |
|-------------------------------|---------------------------------------------------------------|---------------------------------------------------|-------------------------------------|---------------------------------------------|------------------------------------|
| Lubricating agent 44 weight % | Liquid viscosity having a Redwood viscosity at 30°C. (second) |                                                   |                                     |                                             |                                    |
| 40                            | "GAFAC GB-520" *1                                             | "PLUSSIZE J-4" *8                                 | 1.4                                 | 39                                          |                                    |
| 80                            | do.                                                           | do.                                               | 1.5                                 | 37                                          |                                    |
| 150                           | do.                                                           | do.                                               | 1.3                                 | 35                                          |                                    |
| 250                           | do.                                                           | do.                                               | 1.6                                 | 28                                          |                                    |
| 300                           | do.                                                           | do.                                               | 1.5                                 | 27                                          |                                    |
| 500                           | do.                                                           | do.                                               | 1.4                                 | 24                                          |                                    |
| 150                           | "PHOSPHAC L-6" *2                                             | do.                                               | 1.4                                 | 33                                          |                                    |

Table 7—Continued

| Treating agent                                                      |                    | Lubricating agent<br>44 weight %                                         | Self-emulsifying<br>surface active agent<br>50 weight % | Polyacrylic<br>sizing agent<br>6 weight % | Treating<br>agent<br>adhering<br>to yarns<br>(weight %) | Fluff length<br>on<br>cutting yarn<br>(mm.) |
|---------------------------------------------------------------------|--------------------|--------------------------------------------------------------------------|---------------------------------------------------------|-------------------------------------------|---------------------------------------------------------|---------------------------------------------|
| Liquid viscosity having<br>a Redwood viscosity at 30°C.<br>(second) |                    |                                                                          |                                                         |                                           |                                                         |                                             |
| do.                                                                 | "PHOSPHAC O-8"**3  | do.                                                                      | 1.5                                                     | 35                                        |                                                         |                                             |
| do.                                                                 | "GAFAC RS-610"**4  | do.                                                                      | 1.5                                                     | 28                                        |                                                         |                                             |
| do.                                                                 | "GAFAC LO-529"**5  | do.                                                                      | 1.4                                                     | 31                                        |                                                         |                                             |
| do.                                                                 | "GAFAC RD-520Y"**6 | do.                                                                      | 1.2                                                     | 28                                        |                                                         |                                             |
| do.                                                                 | "GAFAC RD-720"**7  | do.                                                                      | 1.5                                                     | 29                                        |                                                         |                                             |
| do.                                                                 | "GAFAC GB-520"     | "NAPS-2"**9                                                              | 1.3                                                     | 24                                        |                                                         |                                             |
| do.                                                                 | do.                | Sodium polyacrylate<br>having a degree of<br>polymerization of<br>900*10 | 1.4                                                     | 38                                        |                                                         |                                             |
| 150                                                                 | "GAFAC GB-520"     | "PLUSSIZE 208C"**11                                                      | 1.5                                                     | 36                                        |                                                         |                                             |
| do.                                                                 | do.                | "MAPOZOL W-1"**12                                                        | 1.4                                                     | 32                                        |                                                         |                                             |
| do.                                                                 | do.                | "MAPOZOL W-6"**13                                                        | 1.5                                                     | 30                                        |                                                         |                                             |
| do.                                                                 | do.                | "MAPOZOL W-412"**14                                                      | 1.3                                                     | 27                                        |                                                         |                                             |

\*1 Trade mark : "GAFAC GB-520", made by Toho Chemical Inc. Co., Ltd.  
 \*2 do. : "PHOSPHAC L-6" (triphosphate, R=C<sub>12</sub>, n=6), made by Toho Chemical Inc. Co., Ltd.  
 \*3 do. : "PHOSPHAC O-8" ( do. , R=C<sub>18</sub>, n=8), do.  
 \*4 do. : "GAFAC RS-610" (mixture of monophosphate and diphosphate, R=C<sub>13</sub>, n=6) do.  
 \*5 do. : "GAFAC LO-529" ( do. , R=nonylphenyl, n=6), do.  
 \*6 do. : "GAFAC RD-520Y" ( do. , R=C<sub>12</sub>, n=4), do.  
 \*7 do. : "GAFAC RD-720" ( do. , R=C<sub>18</sub>, n=7) do.  
 \*8 do. : "PLUSSIZE J<sub>4</sub>" (polyacrylate copolymer), made by Matsumoto Oil & Fat Pharmaceutical Co., Ltd.  
 \*9 do. : "NAPS-2" (polyacrylic acid), do.  
 \*10 do. : made by Katayama Chemical Ind. Co., Ltd.  
 \*11 do. : "PLUSSIZE 208C" (polyacrylate copolymer), do.  
 \*12 do. : "MAPOZOL W-1" ( do. ), do.  
 \*13 do. : "MAPOZOL W-6" ( do. ), do.  
 \*14 do. : "MAPOZOL W-412" ( do. ), do.

## EXAMPLE 9

To a melt-spun, undrawn, semi-dull nylon 6, 6 multifilament yarn consisting of 24 filaments having a denier of 210 there were independently applied the emulsions of treating agents A and B set forth below by rolls according to an ordinary method when taken up at a rate of 1,000 meters per minute so that the amount of the treating agent adhering to the undrawn yarn was about 1.5 percent based on the weight of the yarn. After completion of the treatment the wound-up, undrawn yarn was drawn 3X by usual drawing and twisting machines and wound up on bobbins to give a multifilament yarn having 15 twists per meter and a fluff length of 34 mm. (according to the treating agent A) and 35 mm. (according to the treating agent B), respectively and consisting of 24 filaments having a denier of 70. During the above-described spinning, winding-up, drawing and twisting processes, there was observed no falling off of the polyacrylic sizing agent adhering to the yarn and the yarn traveled very smoothly on the yarn-conveying

devices. Yield of first grade multifilament yarns was 95 percent (according to the treating agent A) and 93 percent (according to the treating agent B), respectively. Then the multifilament yarn was subjected to rough warping process without another twisting of more than 100 twists per meter and sizing, and subsequently to beaming, warp passing and water-jet looming to give 50 pieces of taffeta textile fabrics. During the weaving process there was no falling off of the sizing agent. Rate of weaving operation was 92 percent (according to the treating agent A) and 93 percent (according to the treating agent B), respectively, and the rate was equal to or higher than that with a conventionally sized yarn. The textile fabrics thus obtained were almost free from pear drops and cracks and scouring ability was good. Yield of first grade textile fabrics was 91 percent (according to the treating agent A) and 93 percent (according to the treating agent B), respectively, which was equal to or higher than that with a conventionally sized yarn.

## Treating agent A

- a. Oleyl oleate 40 weight %
- b. Alkylphosphite triester of polyethylene glycol ether having a HLB of 7.3 (Trade mark : "PHOSTAFAT" made by Hoechst A.G.) 50
- c. Polyacrylate sizing agent (Trade mark : "MAPOZOL W-412" made by Matsumoto Oil and Fat Pharmaceutical Co.,Ltd.) 6
- d. sulfated sperm oil (Trade mark : "AK-37" made by Kao Atlas Co.,Ltd.) 4

## Treating agent B

- a. The same as in treating agent A 40 weight %
- b. Alkylphosphate of polyethylene glycol ether having a HLB of 6.9 (Trade mark : "GAFAC GB-520" made by Toho Chemical Inc. Co.,Ltd.) 50
- c. The same as in treating agent A 4
- d. do. 6

The treating agents A and B, each independently dispersed in water to obtain emulsions A and B having a concentration of the treating agent of 16 weight %.

### COMPARATIVE EXAMPLE 1

To a melt-spun, undrawn, semi-dull nylon 6 multifilament yarn consisting of 17 filaments having a denier of 210 there were independently applied, the emulsions of treating agents A and B by rolls when taken up at a rate of 1,000 meters per minute so that the amount of the treating agent adhering to the undrawn yarn was about 1.5 percent based on the weight of the yarn. After completion of the treatment, the wound-up, undrawn yarn was drawn 3X by ordinary drawing and twisting machines, and wound up on bobbins to give a multifilament yarn consisting of 17 filaments having a denier of 70 and having 15 twists per meter and a fluff length on cutting a yarn of 90 mm. with the treating agent A and 93 mm. with the treating agent B. During the spinning, winding-up, drawing and twisting processes, the sizing agent fell off much from the yarn and yield of first grade multifilament yarns was only 14 percent with the treating agent A. On the other hand, with the treating agent B there was observed no falling off of the sizing agent during these processes and yield of first grade multifilament yarns was 90 percent. However weaving was impossible with yarns treated with the treating agents A and B without twisting of more than 100 twists per meter or without ordinary sizing.

was applied the emulsion of treating agent shown below by rolls when taken up at a rate of 1,000 meters per minute so that the amount of the treating agent adhering to the undrawn yarn was 1.6 percent based on the weight of the yarn. After completion of the treatment, the wound-up, undrawn yarn was hot drawn 3X by ordinary drawing and twisting machines, and wound up on bobbins to give a multifilament yarn having 15 twists per meter and consisting of 24 filaments having denier of 75. During the above-described spinning, winding-up, drawing and twisting processes there was observed no falling off of the polyacrylic sizing agent adhering to the yarn and the yarn traveled very smoothly on the yarn-conveying devices. Yield of first grade multifilament yarns was 90 percent. Then the multifilament yarn was subjected to rough warping without another twisting of more than 100 twists per meter and sizing, and subsequently to beaming, warp passing and water-jet looming to give 50 pieces of taffeta textile fabrics. During the weaving process there was observed no falling off of the sizing agent. Rate of weaving operation was 92 percent, and this rate was equal to or higher than that with a conventionally sized yarn. The textile fabrics thus obtained were free from pear drops and cracks. Also scouring ability was good and the yield of first grade textile fabrics was 95 percent, which was equal to or higher than that with a conventionally sized yarn.

| Treating agent A                                                                                                                         | 35 | Treating agent | Weight % |
|------------------------------------------------------------------------------------------------------------------------------------------|----|----------------|----------|
| a. Liquid paraffin having a Redwood viscosity at 30°C. of 25 seconds                                                                     | 30 | 30 weight %    |          |
| b. Alkylphosphate of polyethylene glycol ether having a HLB of 6.9<br>(Trade mark : "GAFAC GB-520" made by Toho Chemical Ind. Co., Ltd.) | 40 |                |          |
| c. Alkylimidazoline<br>(Trade mark : "ELECTROSTRIPPER C" made by Kao Atlas Co., Ltd.)                                                    | 5  |                |          |
| d. Polyacrylate sizing agent<br>(Trade mark : "PLUSSIZE 208C" made by Gao Chemical Ind. Co., Ltd.)                                       | 35 |                |          |
|                                                                                                                                          | 45 |                |          |
| Treating agent B                                                                                                                         | 50 |                |          |
| a. Liquid paraffin having a Redwood viscosity at 30°C. of 250 seconds                                                                    | 60 |                |          |
| b. Polyoxyethylene glycerine ester<br>(Polyoxyethylene : 25 moles)<br>(Trade mark : "K-1161" made by Kao Atlas Co., Ltd.)                | 29 |                |          |
| c. Alkylimidazoline<br>(Trade mark : "ELECTROSTRIPPER C" made by Kao Atlas Co., Ltd.)                                                    | 5  |                |          |
| d. Polyacrylate sizing agent<br>(Trade mark : "PLUSSIZE 208C" made by Gao Chemical Ind. Co., Ltd.)                                       | 6  |                |          |
|                                                                                                                                          | 55 |                |          |

The treating agents A and B, each independently, dispersed in water to obtain emulsions A and B having a concentration of the treating agent of 16 weight %.

### EXAMPLE 10

To a melt-spun, undrawn polyethylene terephthalate consisting of 24 filaments having a denier of 225 there

To a melt-spun, undrawn nylon 6 multifilament yarn consisting of 17 filaments having a denier of 210 there was applied the emulsion of treating agent set forth below by oiling rolls so that the amount of the treating agent adhering to the undrawn yarn was 1.6 percent based on the weight of the yarn. Then the yarn was drawn 3X by a conventional method. The fluff length on cutting the resulting drawn multifilament yarn consisting of 17 filaments having a denier of 70 is shown in Table 8, which indicates high coherency.

Table 9

| Treating agent                                                                                                                                 | weight % |
|------------------------------------------------------------------------------------------------------------------------------------------------|----------|
| a. Mineral oil having a Redwood viscosity at 30°C. of 150 seconds                                                                              | 40       |
| b. Alkylphosphate of polyethylene glycol ether (Polyoxyethylene : 7 moles) (Trade mark : "PLUSSIZE 208 C" made by Gao Chemical Ind. Co., Ltd.) | 50       |
| c. Polyacrylic acid having a degree of polymerization of 1,000                                                                                 | 6        |
| d. Alkylimidazoline (Trade mark : "ELECTROSTRIPPER C" made by Kao Atlas Co., Ltd.)                                                             | 4        |

The treating agent was dispersed in water to obtain an emulsion having a concentration of the treating agent of 16 weight %.

Table 8

| Yarns                                                                               | Fluff length cutting a yarn (mm.) | Remarks                                                                          |
|-------------------------------------------------------------------------------------|-----------------------------------|----------------------------------------------------------------------------------|
| Yarns according to this invention                                                   | 28                                | —                                                                                |
| Yarns according to a conventional method                                            | 133                               | Treated with the emulsion without the phosphate and the polyacrylic sizing agent |
| Sized yarns                                                                         | 14                                | Treated only with the polyacrylic acid sizing agent                              |
| Yarns according to the method disclosed in Japanese Patent Publication No.3319/1971 | 90                                | —                                                                                |

## EXAMPLE 12

To a melt-spun, undrawn nylon 6,6 multifilament yarn consisting of 24 filaments having a denier of 210 there was applied the emulsion of treating agent set forth below by oiling rolls so that the amount of the treating agent adhering to the undrawn yarn was 1.6 percent based on the weight of the yarn. Then the undrawn yarn was drawn 3X by a conventional method. The fluff length on cutting the resulting drawn multifilament yarn consisting of 24 filaments having a denier of 70 is shown in Table 9, which indicates high coherency.

| Treating agent                                                                                                                                 | weight % |
|------------------------------------------------------------------------------------------------------------------------------------------------|----------|
| a. Mineral oil having a Redwood viscosity at 30°C. of 150 seconds                                                                              | 20       |
| b. Butyl stearate                                                                                                                              | 20       |
| c. Alkylphosphate of polyethylene glycol ether (Polyoxyethylene : 7 moles) (Trade mark : "PLUSSIZE 208 C" made by Gao Chemical Ind. Co., Ltd.) | 50       |
| d. Polyacrylic acid having a degree of polymerization of 1,000                                                                                 | 6        |
| e. Sulfated sperm oil (Trade mark : "AK-37" made by Kao Atlas Co., Ltd.)                                                                       | 4        |

The treating agent was dispersed in water to obtain an emulsion having a concentration of the treating agent of 16 weight %.

| 5                                                                                   | Yarns | Fluff length cutting a yarn (mm.) | Remarks                                                                          |
|-------------------------------------------------------------------------------------|-------|-----------------------------------|----------------------------------------------------------------------------------|
| Yarns according to this invention                                                   | 29    | —                                 | Treated with the emulsion without the phosphate and the polyacrylic sizing agent |
| Yarns according to a conventional method                                            | 145   | —                                 | Treated only with the polyacrylic acid sizing agent                              |
| Sized yarns                                                                         | 18    | —                                 | —                                                                                |
| Yarns according to the method disclosed in Japanese Patent Publication No.3319/1971 | 103   | —                                 | —                                                                                |

## EXAMPLE 13

20 To a melt-spun, undrawn polyethylene terephthalate multifilament yarn consisting of 24 filaments having a denier of 175 there was applied the emulsion of treating agent set forth below by oiling rolls so that the amount of treating agent adhering to the undrawn yarn was 1.6 percent based on the weight of the yarn. Then the yarn was hot drawn 3.5X by a conventional method. The fluff length on cutting the resulting drawn multifilament yarn consisting of 24 filaments having a denier of 50 is shown in Table 10, which indicates high coherency.

Table 10

| 35                                                                                  | Yarns | Fluff length cutting a yarn (mm.) | Remarks                                                                          |
|-------------------------------------------------------------------------------------|-------|-----------------------------------|----------------------------------------------------------------------------------|
| Yarns according to this invention                                                   | 30    | —                                 | Treated with the emulsion without the phosphate and the polyacrylic sizing agent |
| Yarns according to a conventional method                                            | 128   | —                                 | Treated only with the polyacrylic acid sizing agent                              |
| Sized yarns                                                                         | 19    | —                                 | —                                                                                |
| Yarns according to the method disclosed in Japanese Patent Publication No.3319/1971 | 93    | —                                 | —                                                                                |

| Treating agent                                                                                                                               | weight % |
|----------------------------------------------------------------------------------------------------------------------------------------------|----------|
| a. Mineral oil having a Redwood viscosity at 30°C. of 300 seconds                                                                            | 30       |
| b. Oleyl oleate                                                                                                                              | 15       |
| c. Alkylphosphate of polyethylene glycol ether (Polyoxyethylene : 7 moles) (Trade mark : "PLUSSIE 208C" made by Gao Chemical Ind. Co., Ltd.) | 40       |
| d. Polyacrylic acid having a degree of polymerization of 1,000                                                                               | 8        |
| e. Alkylphosphate (Trade mark : "A-72" made by Takemoto Oil & Fats Co., Ltd.)                                                                | 7        |

60 The treating agent was dispersed in water to obtain an emulsion having a concentration of treating agent of 16 weight %.

65 What is claimed is:

1. A synthetic thermoplastic multifilament yarn having at most 100 twists per meter carrying about 0.5 to 3.0 percent, based on the weight of the yarn, of a treating agent comprising about 5 to 68 percent by weight of a liquid, synthetic yarn lubricating agent, about 30 to 80 percent by weight of a self-emulsifying organic

phosphorus-containing surface active agent having a HLB of from about 4 to 15 and about 2 to 15 percent by weight of a polyacrylic sizing agent, the polyacrylic size being present in about 0.02 to 0.25 percent, based on the weight of the yarn.

2. The synthetic thermoplastic multifilament yarn of claim 1 wherein the amount of the polyacrylic sizing agent adhering to the yarn is from about 0.075 to 0.175 percent based on the weight of the yarn.

3. The synthetic thermoplastic multifilament yarn of claim 1 wherein the amount of the polyacrylic sizing agent in the treating agent is about 4 to 8% by weight.

4. The synthetic thermoplastic multifilament yarn of claim 1 wherein said treating agent additionally contains an antistatic agent.

5. A process for producing synthetic thermoplastic multifilament yarns having improved coherency and smoothness which comprises, prior to drawing, treating undrawn synthetic thermoplastic multifilament yarns with a treating agent comprising about 5 to 68 percent by weight of a liquid, synthetic yarn lubricating agent, about 30 to 80 percent by weight of a self-emulsifying organic phosphorus-containing surface active agent

having a HLB of from about 4 to 15 and about 2 to 15 percent by weight of a polyacrylic sizing agent so that the amount of said treating agent adhering to said yarns is from about 0.5 to 3.0 percent based on the weight of the yarns and the amount of said polyacrylic sizing agent adhering to said yarns is from about 0.02 to 0.25 percent based on the weight of the yarns, and thereafter hot drawing and winding said yarns.

6. The process of claim 5 wherein the treating agent contains additionally an antistatic agent.

7. The process of claim 5 wherein the treating agent is employed in the form of a dispersion in water with a concentration of said treating agent being from about 10 to 25 percent by weight.

8. The process of claim 7 wherein the dispersion in water is applied to the undrawn multifilament yarns which is being taken up at a rate of from about 600 to 5,000 meters per minute.

9. The process of claim 8 wherein the synthetic thermoplastic material constituting said yarn is polyamide, polyester or polypropylene.

\* \* \* \* \*